

## UNITED STATES PATENT OFFICE

2,248,961

## COATING COMPOSITION

Herbert C. Comstock, Mount Kisco, N. Y.

No Drawing. Application June 21, 1938, Serial  
No. 214,938

3 Claims. (Cl. 134—1)

This invention relates to surface coatings and more particularly to the type which may be applied to a surface in liquid form by brushing, spraying or dipping.

The invention further relates to a surface covering composition that may be applied to and bonded with practically any surface but is particularly well suited for application to metal surfaces as a rustproofing treatment. Not only does the invention comprehend a rustproofing material but the composition by simple application to surfaces, and particularly, metal surfaces, is admirably suited as a primer or surfacer for paint, varnish, lacquer, synthetic and other enamels and finishes.

For example, in the automobile industry it has been common practice, in treating automobile body surfaces for the application of the top coats or finishing lacquers, to apply a number of aggregate coats, followed by a sanding or smoothing operation. According to the usual practice after the body surface has been cleaned, a rust inhibitor coat is applied which is baked or otherwise dried. Next is applied a primer coat which also requires baking. Then, from two to three coats of pigmented surfacer or filler (sometimes more, according to the price at which the car is to be sold) are applied, and these in turn are baked. This is followed by a sanding operation to smooth the surface preparatory to receiving the finishing coats.

It is one of the objects of this invention to eliminate a number of aforementioned operations in preparing metal surfaces, such as automobile bodies, for lacquering or finishing coats while at the same time producing a rustproofing treatment. Furthermore, not only is an effective rustproofing treatment provided but the surface resulting from a single application of the composition comprehended by the invention is relatively smooth and non-porous as compared to the surfaces produced by the processes hereinabove mentioned. Consequently, according to the present invention very little sanding is required preparatory to application of the finishing coats. Moreover, being less porous than pigmented fillers, the primer surfacer produced in accordance with the present invention requires a less number of finishing lacquer coats for the desired finish, which can be brought more easily to a higher brilliancy of luster and finish than could be produced over pigmented surfacers or undercoats.

The invention, however, is not limited to automobile finishing but finds utility as a rustproof-

ing treatment per se without additional coatings of lacquer or other finishes. According to the invention the composition also may serve as a vehicle for pigments to be used in place of or in conjunction with linseed oil or other common vehicles to improve the appearance, spreading and lasting qualities of the paints so compounded.

10 Stated generally, the invention consists in providing a composition by compounding a medium oil varnish with a material which gives to the resulting composition a sustained flexibility, a material inert to oxidation to lend acid and alkali resistivity, a drying or oxidizable oil and a quick evaporating material which serves to reduce the surface tension of the mixture when applied whereby it will readily penetrate into pores, cracks and crevices to give bonding qualities but which will quickly evaporate after the composition is applied to a surface to be coated.

15 The invention further consists in forming a product having the general characteristics, the new and useful applications, and the several features of utility hereinafter described and in the 20 new and novel features of operation and the new and original arrangements and combinations of steps in the process hereinafter set forth and more particularly as defined in the annexed claims.

25 In a preferred form of this invention a surface covering composition is formed by suitably compounding a medium oil varnish with predetermined amounts of beeswax, paraffin wax, boiled linseed oil and mineral spirits. When 30 properly compounded the composition thus formed may be variously modified depending upon the use to which it is to be put. For convenience of description the base material so formed is hereinafter called "rustproofing-primer-vehicle". It will be understood that the rustproofing-primer-vehicle may be used for certain purposes without further modification while other 35 purposes may require additions or modifications to the rustproofing-primer-vehicle depending upon the use for which it is intended.

40 The following example is set forth as illustrative of one embodiment of the invention. A 45 rustproofing-primer-vehicle may be prepared by heating and stirring in a double jacketed boiler one and one-quarter gallons of medium oil varnish, three pounds of beeswax, and one-half pound of paraffin wax until all of these materials are thoroughly dissolved and intimately mixed. The temperature should be brought to approximately 190° F. during this operation. After the

foregoing ingredients are formed into a homogeneous mixture then add to the mixture with constant stirring two and one-quarter gallons of boiled linseed oil, one gallon of mineral spirits and two and one-quarter gallons of medium oil varnish. The mixture should be well stirred and the temperature maintained at approximately 170° F. Then add to this heated mixture eighteen and one-half gallons of mineral spirits. This should result in approximately a twenty-five gallon batch. The batch should then be occasionally stirred for about ten minutes and then re-heated to a temperature of about 198° F. and allowed to stand for about 40 minutes at that temperature.

It will be understood that in this connection "medium oil varnish" comprehends the varnish known generally in the trade by that name. It is a varnish which comprises twenty to thirty gallons of oil to each 100 pounds of gums or resins. I have found that a varnish containing 100 pounds of phenolic resins to twenty-four gallons of China-wood oil produces very desirable results. The beeswax may be of a good commercial grade having a melting point of 140° to 150° F. The paraffin should be of a good commercial grade having a melting point from 120° F. to 130° F. The mineral spirits which I have found to give best results has a distillation range of from 300°-310° F. (initial boiling point) to 390°-400° F. (end point). For purposes of safety the flash point should not be less than 100° F.

The rustproofing-primer-vehicle prepared in accordance with the foregoing, after cooling is then ready for use as a rustproofing coating which may be applied directly to a clean metal surface and allowed to dry at atmospheric temperature or oven dried as desired. The coating thus applied constitutes an excellent rustproofing treatment. It will be found to have penetrated the pores, cracks and crevices of the metal and has exceptional adhesive and bonding characteristics. It will remain in a sustained state of flexibility and will remain transparent.

If desired, the rustproofing-primer-vehicle may be prepared according to the following formula:

|                                    | Per cent<br>by weight |
|------------------------------------|-----------------------|
| Medium oil varnish                 | 14.7                  |
| Beeswax                            | 1.7                   |
| Paraffin wax                       | .3                    |
| Boiled linseed oil                 | 10.0                  |
| Mineral spirits—sufficient to make | 100                   |

I have found that the following method of compounding produces the desired results. To about half of the medium oil varnish add the beeswax and paraffin and heat to about 190° F. and stir until the waxes are thoroughly dissolved, then add the linseed oil with constant stirring until the mixture is homogeneous. Then add about a tenth of the mineral spirits and the remainder of the medium oil varnish. Heat this mixture to about 170° F. and add the remainder of the mineral spirits. Stir the mixture thoroughly for about ten minutes, reheat to about 198° F. and allow to stand for about 40 minutes at that temperature. This mixture is then cooled.

To make a one coat transparent, non-pigment rustproofing primer and surfacer, that is, as a base coat for applying lacquer or other finishes, mix two parts of the rustproofing-primer-vehicle with one part of medium oil varnish. A composition so made is herein referred to as a "non-

pigment primer and surfacer". Its formula on a percentage by weight basis will be as follows:

|                    | Per cent       |
|--------------------|----------------|
| Medium oil varnish | 17.6           |
| Beeswax            | 1.6            |
| Paraffin wax       | .3             |
| Boiled linseed oil | 9.6            |
| Mineral spirits    | Balance to 100 |

While the preferred formula for the non-pigment primer and surfacer has been set forth the invention is not intended necessarily to be limited to the precise percentages as it has been found that the amount of beeswax may vary from about 1% to about 3% with desirable results and the paraffin wax may vary from about 0.1% to about 1.0% with percentages of the other ingredients remaining approximately the same.

The use of the non-pigment primer and surfacer will be described in connection with finishing an automobile body although it will be apparent as the description proceeds that other metal surfaces may be similarly treated.

After the surface of the body has been cleaned in the usual manner one coat of the non-pigment primer and surfacer is sprayed on the body. The body is then oven dried for approximately one hour at about 200° F. Or, if desired, this oven drying may be accelerated by increasing the temperature. If the drying temperature is increased to 300° F. the requisite drying will require only about fifteen minutes.

After drying, the non-pigment primer and surfacer will require very little, if any, sanding as it will be found that the surface dries smooth and a non-porous coating is tenaciously bonded to the metal by reason of its having penetrated into pores and crevices. The body is then ready for application of lacquer finishes in the usual way and it has been found that three sprayed coats of the latter will be sufficient whereas in processes now commonly used over porous or pigmented undercoats, more coats of lacquer are generally required.

Consequently, the invention effects economies, in floor space, ovens, number of operations, and time schedules in addition to savings in materials while at the same time affording an effective rustproofing treatment by a protective coating which will have excellent adhesive and flexibility characteristics.

In addition to the foregoing mentioned uses the rustproofing - primer - vehicle composition comprehended by the invention may serve as a vehicle for white lead; red lead and other paint pigments. For example, red lead mixed with the rustproofing-primer as the vehicle when used as a prime or base coat (outdoors, as on structural steel bridges) will dry over night free from tack, and cover more than twice the surface area, than an equal quantity of the same red lead mixed with a like amount of linseed oil used as the vehicle. The vehicle will penetrate the crevices and pores in the steel and the paint so made provides a most effective rust repellent base.

The term "rustproofing" as herein used is intended as a word of description and to have its usual connotation as generally understood in the trade since by its nature it is a relative term. Herein, it is intended to connote that characteristic of inhibiting oxidation for abnormally extended periods of time as it is generally known that all oxidizable metals, if exposed to oxidants indefinitely, will finally become oxidized to a greater or less degree.

Likewise, other terms and expressions which have been employed are used as terms of description, and there is no intention, in the use of such terms and expressions, of excluding equivalents of the features described, but it is recognized that various modifications are possible within the scope of the claims hereto appended.

What is claimed is:

1. A liquid vehicle for paint pigments comprising a mixture of ingredients in approximate proportions as follows: three and one-half gallons of medium oil varnish containing not more than eleven and six-tenths pounds of gums and resins, three pounds of beeswax having a melting point of 140° to 150° F., one-half pound of paraffin wax having a melting point from 120° to 130° F., two and one-quarter gallons of boiled linseed oil and nineteen and one-half gallons of mineral spirits having an initial boiling point of 300°-310° F. and an end point of 390°-400° F.

2. A composition consisting of medium oil varnish approximately 14.7% by weight, beeswax having a melting point 140°-150° F. approximately 1.7% by weight, paraffin wax approxi-

10 mately 0.3%, boiled linseed oil approximately 10%, balance mineral spirits having an initial boiling point and an end point of about 300° F. and 400° F. respectively to make 100% by weight, said composition being in the form of a homogeneous liquid and being characterized by drying rapidly when applied to clean metal surfaces leaving a transparent, permanently flexible coating tenaciously bonded thereto.

15 3. A composition comprising medium oil varnish approximately 17.6% by weight, beeswax having a melting point 140°-150° C. approximately 1.6% by weight, paraffin wax having a melting point 120°-130° F. approximately 0.3% by weight, boiled linseed oil approximately 9.6% by weight, balance mineral spirits having an initial boiling point 300°-310° F. and an end point 390°-400° F. to make 100% by weight, said composition being characterized by its property of drying rapidly 20 when applied to a clean metal surface leaving a single transparent flexible primer and surfacer coating tenaciously bonded to said metal surfaces.

HERBERT C. COMSTOCK.